# EUROPEAN PATENT SPECIFICATION

(11) **EP 0 311 860 B1**
(45) Date of publication and mention of the grant of the patent: **03.07.1996**
(21) Application number: 88116222.6
(22) Date of filing: 30.09.1988
(51) Int. Cl.: D01F 8/06, D04H 1/54

(54) **Nonwoven fabric made of heat bondable fibers**
Vliesstoff hergestellt aus Schmelzklebkompositfasern
Non-tissé fabriqué à partir de filaments soudables à chaud

(30) Priority: 02.10.1987 JP 250409/87
(43) Date of publication of application: 19.04.1989
(73) Proprietor: UNITIKA LTD., Amagasaki-shi Hyogo-ken (JP)
(72) Inventor: Kubo, Eiichi, 23, Uji Kozakura Uji-shi Kyoto (JP); Sasaki, Shingo, Okazaki-shi Aichi-ken (JP)
(74) Representative: Le Vrang, Klaus

(56) References cited:
- EP-A- 0 132 110
- EP-A- 0 239 080
- GB-A- 2 180 543
- JP-A- 6 110 583
- JP-B-61 010 583
- CHEMICAL ABSTRACTS, vol. 97, no. 24, 13th December 1982, abstract no. 202486b, Columbus, Ohio, US; & JP-A-82 106 563
- Encyclopedia of Polymer Science and Engineering, vol. 6; John Wiley & Sons, New York (US); p. 830 (1986)
- Encyclopedia of Polymer Science and Engineering, vol. 6; John Wiley & Sons, New York (US); p. 423 (1986)

## Description

### FIELD OF THE INVENTION

The present invention relates to a nonwoven fabric made of a core-sheath type composite heat-bondable staple fiber having superb heat-bondability and a nonwoven fabric made of said fiber.

### BACKGROUND OF THE INVENTION

A nonwoven fabric made of composite type heat-bondable staple fiber has been known, disclosed in DE-A 33 23 467. This nonwoven fabric is obtained by heat-treating a mixture of fibers containing not less than 25 weight percent of a heat-bondable composite fiber which comprises a first component consisting of 50-100 weight percent of linear low density polyethylene and 50-0 weight percent of polyethylene different therefrom, and a second component in the form of a fiber-forming polymer (polypropylene, polyester, polyamide or the like) exhibiting a melting point which is more than 30° C higher than that of these polyethylenes, the heat-treatment being performed at a temperature above the melting point of said first component but below the melting point of said second component.

The desire of the industry for a nonwoven fabric having a high strength and a soft hand is very high; the composite type heat-bondable fiber disclosed in said DE-A 33 23 467 is capable of offering a nonwoven fabric having a soft hand. However, it has the drawback that it is lacking in the adhesion to fibers of other materials than polyethylene, in which case it is necessary to increase the amount of heat-bondable fiber, hardly providing a nonwoven fabric which is soft in terms of hand.

### APPRECIATION OF PRIOR ART

The GB-A-2180543 discloses a nonwoven fabric made of a core-sheath type heat-bondable fiber. It has a fiber forming component as its core component and a bondable component as its sheath component. Incidentally, in case of forming a nonwoven fabric especially using core-sheath type short fibers, the strength of each fiber per se and the force of the adhesion between each fibers are required to be sufficiently high. Furthermore it is necessary to securely incorporate the core component with the sheath component so that they will not come off each other.

To be particular, the heat-bondable fiber disclosed in GB-A-2180543 has a sheath component made of for example unmodified polyolefin, in order to improve the force of adhesion between fibers. Moreover, in order to improve the force of adhesion between the sheath component and the core component from coming off each other, the core component is made of a mixture containing a copolymer having good adhesion to the sheath component.

However, there is such a problem that when a core component comprises a copolymer, the strength of the core component becomes insufficient, consequently the strength of the core sheath type fiber per se becoming insufficient.

### OBJECT OF THE DISCLOSURE

It is an object of the present invention to present a nonwoven fabric made of a heat-bondable fiber which is high in adhesion even when it adheres to a dissimilar fiber, high in strength of the fiber per se and further free from the possibility of the core and sheath components coming off each other, and which is capable of providing a nonwoven fabric having an improved good hand.

A non-woven fabric according to the invention is made of a heat-bondable staple fiber in the form of a core-sheath type composite fiber comprising a core component and a sheath component which covers the periphery of said core component, said sheath component being formed of ethylene copolymer consisting of ethylene and other comonomer which consists of at least one member selected from the class consisting of an unsaturated carboxylic acid, a derivative from said unsaturated carboxylic acid and a carboxylic acid anhydride of said unsaturated carboxylic acid, said core-sheath type composite fiber having a single fiber fineness of less than 8 deniers, said nonwoven fabric containing said heat-bondable fiber and being heat treated at a temperature below the melting point of the core component, said core component consisting of fiber forming polymer, said fiber-forming polymer having a melting point which is more than 30°C higher than that of the ethylene copolymer of said sheath component, the content of said comonomer is greater than 0.1 mole percent; and the weight percentage of said heat-bondable fiber in said non-woven fabric is at least 15 weight percent.

Said nonwoven fabric is characterised in that the melt index value of said sheath component is I to 50 g/10 minutes as measured by the ASTM D-1238(E), the content of said comonomer is in a range of more than 0.79 mole percent, but no more than 5.0 mole percent, and said fiber forming polymer consists of polyethylene terephthalate, polypropylene or nylon 6.

A nonwoven fabric according to the invention, which contains at least 15% of the heat-bondable fiber of the above-described composition, has been heat-treated at a temperature lower than the melting point of said core component.

The comonomer of ethylene copolymer in the invention, as described above, is an unsaturated carboxylic acid, a derivative from said carboxylic acid, or a carboxylic acid anhydride. Coming under the category of such comonomer are unsaturated carboxylic acids, such as acrylic acid and methacrylic acid; acrylic esters, such as methyl acrylate, ethyl acrylate, butyl acrylate, 2-ethylhexyl acrylate, and 2-hydroxyethyl acrylate; methacrylate esters, such as methyl methacrylate, ethyl methacrylate, butyl methacrylate 2-ethylhexyl methacrylate; and unsaturated carboxylic acid anhydrides, such as maleic acid anhydride and itaconic acid anhydride. The ethylene copolymer of the invention contains one or more such comonomers; thus, these comonomers may be suitably combined. Further, the ethylene copolymer of the invention may be a copolymerisate of ethylene and said carboxylic acid compound in alternate, random or block form or mixture of such forms.

The copolymerization ratio of the comonomer mole to ethylene is restricted to 0.1-5.0 percent with respect to ethylene from the standpoint of physical properties of the copolymer ethylene. In the case where the copolymerization ratio is less than 0.1 mole percent, the adhesion to other fibers is low as in the case of polyethylene alone, with the result that a nonwoven fabric of low strength can only be obtained. On the other hand, if the copolymerization ratio is greater than 5.0 mole percent, the adhesion to other fibers becomes higher, but the melting point or softening point of the ethylene copolymer polyethylene becomes extremely low, which is not desirable from the standpoint of heat resistance when a nonwoven fabric is formed. The reason for restricting the melt index value of the ethylene copolymer to 1-50 g/10 minutes as measured by ASTM D-1238(E) is that in the case of an ethylene copolymer whose melt index value is less than 1 g/10 minutes, the fluidity associated with melt spinning is degraded to the extent that a composite fiber cannot be produced unless the spinning speed is drastically decreased.

On the other hand, if the melt index value exceeds 50 g/10 minutes, this is not desirable since this decreases the strength of the composite fiber. It is necessary that the melting point of the core component of the composite type heat-bondable fiber be more than 30°C higher than the melting point of the ethylene copolymer of the sheath component. To obtain a fabric satisfactory in strength, it is necessary that the heat-bondable fiber be sufficiently melted in the heat treatment process and that after the heat treatment, the configuration of the composite fiber be sufficiently retained. To this end, the difference in melting point between the core and sheath components must be at least 30°C. If there is a difference of more than 30°C therebetween, the configuration retention of the composite fiber will be uniform and the sheath component will be melted in the heat treatment process; therefore, heat treatment conditions which provide compatibility between strength and hand for a nonwoven fabric to be produced can be easily selected.

As for the fiber-forming polymer which constitutes the core component, this is polypropylene, polyester and polyamide, which can be melt-spun. The composite type heat-bondable fiber in the present invention is a composite fiber having a cross-sectional shape in which ethylene copolymer covers the fiber-forming polymer. As for the composition ratio, it is preferable that the amount of the ethylene copolymer in the sheath component be 20-80 weight percent and the amount of the fiber-forming polymer in the core component be 80-20 weight percent. In the case where the amount of the ethylene copolymer of the sheath component is less than 20 weight percent, the strength of the resulting nonwoven fabric is high but the force of adhesion of a mixture to other fibers for making a nonwoven fabric is low; thus, only a nonwoven fabric of low strength can be obtained. On the other hand, if the amount of the ethylene copolymer of the sheath component exceeds 80 weight percent, the force of adhesion in the nonwoven fabric is high but the strength of the fiber itself is low; thus, the nonwoven fabric is of low strength.

The fiber of the invention is a composite fiber whose single fiber fineness is less than 8 deniers. That is, the composite type heat-bondable fiber of the invention is suitable for forming a nonwoven fabric which is required to be particularly soft; thick single fiber would lead to high stiffness and undesirable hand. Therefore, the invention is not directed to thick fibers whose fineness exceeds 8 deniers. In addition, the ethylene copolymer which is the sheath component may have mixed therewith such a polyolefin as polyethylene or polypropylene or may have added thereto a hygroscopic agent, a delusterant, a pigment, a stabilizer and/or a flame retardant.

The composite type heat-bondable fiber of the invention can be produced by using a composite spinning device known in the art. The melt spinning temperature for the sheath component is 180-280° C, preferably 190-250° C, while the melt spinning temperature for the core component may be set according to the conditions for spinning the fiber-forming polymer alone selected as the core component.

The spun, non stretched composite fiber may go without a stretching process in the case where its single fiber fineness is less than 8 deniers; however, usually the resulting non stretched fiber is cold-stretched to 2-8 times the original length at a temperature which is above the room temperature but below the melting point of the sheath component, to provide a composite type heat-bondable fiber.

In the present invention, a group of fibers for forming a nonwoven fabric is composed of either a composite type heat-bondable fiber of less than 8 deniers or a mixture of said heat-bondable fiber and other fibers with a finenesss of less than 8 deniers, said mixture containing at least 15 weight percent of said heat-bondable fibers with respect to the total amount of the mixed fibers. As for said other fibers, it is possible to use any fibers that will neither melt nor greatly shrink during heat treatment for nonwoven fabric production and that satisfy the aforesaid fineness condition. For example, one or two or more members selected from the group consisting of natural fibers such as cotton and wool, semi-synthetic fibers such as viscose rayon and cellulose acetate, and synthetic fibers such as polyolefin fibers such as polyethylene and polypropylene, polyamide fiber, polyester fiber and acrylic fiber may be suitably selectively used in an amount which is less than 85 weight percent with respect to the total amount of the mixed fibers. If the amount of the composite type heat-bondable fiber in the mixed fibers is less than 15 weight percent, this is undesirable as the strength of the nonwoven fabric decreases. The reason why the fineness of other fibers to be mixed with said composite type heat-bondable fiber is restricted to less than 8 deniers is that if a fiber having a fineness greater than this value, it is impossible to obtain a nonwoven fabric of good hand.

As for a method of forming a composite type heat-bondable fiber alone or a mixture of said composite fiber and other fibers into a web, use may be made of known methods used for producing nonwoven fabrics in general, such as carding, air laying, wet paper screening. Then, the resulting group of fibers in web form is heat-treated at a temperature below the melting point of the core component of the composite fiber, whereby a nonwoven fabric is obtained.

As for a machine for heat treatment, use may be made of heat treating devices including such dryers as a hot air dryer and a suction drum dryer, and such hot rolls as a flat calender roll and an embossing roll.

Whether the heat-bondable fiber of the invention is used for a nonwoven fabric or it is mixed with other fibers to serve as a binder, a nonwoven fabric of good hand can be obtained since in either case the force of adhesion between fibers is high. For this reason, it has a wide application in covering sheets for disposable diapers and sanitary articles and in the medical field.

### DESCRIPTION OF EXAMPLES

The invention will now be described in more concrete with reference to examples thereof. Methods for measuring the tensile strength, compression bending rigidity (an index indicating softness) and weight of nonwoven fabrics referred to in the examples will first be described.

### (1) Tensile Strength

The maximum tensile strength of a 30 mm wide and 100 mm long test piece was measured according to JIS L-1096 Strip Method.

### (2) Compression Bending Rigidity (Softness)

A 50 mm x 100 mm test piece was formed into a 50 mm high cylinder having a circumference of 100 mm, and said cylinder placed on a flat plate type load cell was loaded under compression; the maximum compression load applied was measured.

### (3) Weight

Determined according to JIS P-8142.

### (4) Overall Appraisal

Appraised on the basis of both tensile strength and compression bending rigidity. The appraisal marks used hereinafter are as follows:
Appraisal Marks
- 0: Good
- x: Bad

### (Example 1, Comparative Example 1)

Melt extrusion was performed by using as a sheath component ethylene copolymer whose melt index value measured by ASTM D-1238(E) was 10g/10 minutes and whose melting point measured by DSC was 104.6° C and as a core component polyethylene terephthalate whose intrinsic viscosity (η) measured in a phenol/tetrachloroethane (ratio, 1:1) mixed solvent at 20° C was 0.70 and whose melting point measured by DSC was 255° C, and using a composite fiber melt spinning device with a spinneret having 390 holes, at a melting temperature of 230° C for the ethylene copolymer and a melting temperature of 285°C for the polyethylene terephthalate, a single hole delivery rate of 1.5 g/min, the ethylene copolymer /polyethylene terephthalate composite ratio being 50:50. After cooling, the fiber was taken up at a rate of 1100 m/min. The resulting composite non stretched fiber was stretched at a stretch temperature of 85°C and a stretch factor of 3.5 times and crimped by a stuffer type crimper, whereupon it was cut into lengths of 51 mm to produce a staple fiber whose single fiber fineness was 3.5 deniers.

The yarn properties of the resulting staple fiber are shown in Table 1.

Subsequently, this composite fiber staple was fed to a carding machine to form a web having a weight of 15 g/m², and the web was then heat-treated at 120°C by using a suction dryer to form a nonwoven fabric. The properties of the nonwoven fabric obtained are shown in Table 2.

Next, as a comparative example 1, spinning, stretching and crimping of a core-sheath type composite fiber were performed in the same manner as that of Example 1 by using low density polyethylene whose melt index measured by ASTM D-1238(E) was 10 g/10 minutes and whose melting point measured by DSC was 105°C as a sheath component instead of using the ethylene copolymer of Example 1.

The yarn properties of the resulting composite heat-bondable fiber are shown in Table 1. Subsequently, said heat-bondable fiber was formed into a nonwoven fabric in a manner similar to that of Example 1. The properties of the nonwoven fabric obtained are shown in Table 2.

### (Example 2, Comparative Example 2)

Staple fiber consisting of a composite heat-bondable fiber containing a sheath component formed of the ethylene copolymer obtained in Example 1 and a core component formed of polyethylene terephthalate was fed to a carding machine to form a web having a weight of 15 g/m2, said web being heat-treated by calender rolls comprising a metal hot roll and a rubber roll at a roll temperature of 100° C and a line pressure of 35 kg/cm, whereby a nonwoven fabric was obtained. The performance of this nonwoven fabric is shown in Table 2.

As a comparative example 2, a web was produced in the same manner as that of Example 2 by using staple fiber consisting of a composite heat-bondable fiber containing a sheath component formed of the low density polyethylene obtained in Comparative Example 1 and a core component formed of polyethylene terephthalate, said web being then formed into a nonwoven fabric under the calender conditions of Example 2. The performance of the nonwoven fabric obtained is shown in Table 2.

### (Example 3)

Melt extrusion was performed by using as a sheath component the ethylene copolymer used in Example 1 and as a core component polypropylene whose melt flow rate measured by ASTM D-1238(L) was 15 g/10 minutes and whose melting point measured by DSC was 165° C and using a composite spinning device similar to the one used in Example 1, at a melt spinning temperature of 230° C for the ethylene copolymer , a melt temperature of 270° C for the polypropylene, a single hole delivery rate of 2.0 g/min, the ethylene copolymer polypropylene composite ratio being 50:50 by weight. After cooling, the fiber was taken up at a rate of 1100 m/min. The resulting composite non stretched fiber was stretched at a stretch temperature of 70° C and a stretch ratio of 3.5 times and crimped by a stuffer type crimper, whereupon it was cut into lengths of 51 mm to produce a staple fiber whose single fiber fineness was 3.5 deniers. A nonwoven fabric was formed in the same manner as that of Example 1 by using the staple fiber obtained. The properties of this composite heat-bondable fiber are shown in Table 1 and the properties of the nonwoven fabric are shown in Table 2.

### (Examples 4-5, Comparative Examples 3-4)

Nonwoven fabrics were formed in the same manner as that of Example 1, each by using a mixture of the staple fiber consisting of the heat-bondable fiber of Example 1 and another fiber. As for the mixing ratio, the mixture (Example 4) contained 15 parts of the heat-bondable fiber and 85 parts of PET, and the mixture (Example 5) contained 15 parts of the heat-bondable fiber and 85 parts of polypropylene. The properties of the resulting nonwoven fabrics are shown in Table 3.

For comparison with said Examples 4 and 5, nonwoven fabrics were formed in the same manner as that of Example 1, each by using a mixture of the heat-bondable fiber of Comparative Example 1 and another fiber. As for the mixing ratio, the mixture (Comparative Example 3) contained 20 parts of heat-bondable fiber and 80 parts of PET and the mixture (Comparative Example 4) contained 20 parts of heat-bondable fiber and 80 parts of polypropylene. The properties of the nonwoven fabrics are shown in Table 3.

### (Examples 6-7)

Nonwoven fabrics were obtained, each by mixing the heat-bondable fiber of Example 3 with another fiber and passing the mixture through a carding machine in the same manner as in example 1 to form a web, which was then heat-treated by the calender roll method at a roll temperature of 100° C and a line pressure of 35 kg/cm in the same manner as that of Example 2. The properties of said nonwoven fabrics are shown in Table 3.

### (Examples 8-10)

Melt extrusion was performed by using as a sheath component the ethylene copolymer used in Example 1 and as a core component nylon 6 polymer whose relative viscosity ηᵣₑ₁ measured by an Ostwald viscometer by dissolving 1.0 g of the polymer in 100 cc of 96% concentrated sulfuric acid was 2.6 and whose melting point measured by DSC was 220° C, and by using a spinneret having 390 holes, at a melting temperature of 230° C for the ethylene copolymer and a melting temperature of 270° C for the nylon 6 polymer, a single hole delivery rate of 2.0 g/min, the ethylene copolymer/nylon 6 polymer composite ratio being 50:50 by weight. After cooling, the fiber was taken up at a rate of 1100 m/min. The resulting composite non stretched fiber was stretched at a stretch temperature of 80°C and a stretch ratio of 5.5 times and crimped by a stuffer type crimper, whereupon it was cut into lengths of 51 mm to produce a staple fiber whose single fiber fineness was 3.5 deniers.

The resulting staple fiber was mixed with another fiber and passed through a carding machine in the same manner as that of Example 1 to form a web, which was then heat-treated at a temperature of 120°C by a suction drum drier to provide a nonwoven fabric. The properties of the composite type heat-bondable fiber are shown in Table 1 and the properties of the nonwoven fabrics obtained are shown in Table 3.

### (Examples 11-12)

Composite type heat-bondable fiber was produced under the same conditions as in Example 1 except using as a sheath component ethylene copolymer which contained 3 mole percent of acrylic acid and whose melt index measured by ASTM D-1238(E) was 20 g/10 minutes and whose melting point measured by DSC was 96.2° C. The heat-bondable fiber obtained was mixed with another fiber and the mixture was formed into a web in the same manner as that of Example 1 by a carding machine, said web being then heat-treated at a temperature 120° C by the suction drum dryer method to provide a nonwoven fabric. The properties of the composite type heat-bondable fibcr are shown in Table 1, and the performance of the nonwoven fabrics obtained are shown in Table 3.

### (Examples 13-14)

Composite type heat-bondable fiber was produced under the same conditions as in Example 1 except for using as a sheath component copolymer polyethylene which contained 0.5 mole percent of acrylic acid anhydride and 1.5 mole percent of ethylacrylate serving as-comonomers of ethylene and whose melt index measured by ASTM D-1238(E) was 5 g/10 minutes and whose melting point measured by DSC was 107° C. The heat-bondable fiber obtained was mixed with another fiber and the mixture was formed into a web in the same manner as in Example 1 by a carding machine, said web being then heat-treated at a temperature 120° C by the suction drum dryer method to provide a nonwoven fabric. The properties of the composite type heat-bondable fiber are shown in Table 1, and the properties of the nonwoven fabrics obtained are shown in Table 3.

As is clear from Table 3, in the case where the heat-bondable fiber of the present invention was mixed with another fiber to form a nonwoven fabric, there was obtained a nonwoven fabric whose tensile strength was high even if the amount of the heat-bondable fiber in the mixture was low because its high force of adhesion to other fibers and whose hand feels soft. In addition, a nonwoven fabric formed 100 percent of the heat-bondable fiber of the invention had high tensile strength and soft hand.

## Claims

1. A non-woven fabric made of a heat-bondable staple fiber in the form of a core-sheath type composite fiber comprising:
a core component and a sheath component which covers the periphery of said core component;
said sheath component being formed of ethylene copolymer consisting of ethylene and other comonomer which consists of at least one member selccted from the class consisting of an unsaturated carboxylic acid, a derivative from said unsaturated carboxylic acid and a carboxylic acid anhydride of said unsaturated carboxylic acid;
said core-sheath type composite fiber having a single fiber fineness of less than 8 deniers;
said nonwoven fabric containing said heat-bondable fiber and being heat treated at a temperature below the melting point of the core component;
said core component consisting of fiber forming polymer,
said fiber-forming polymer having a melting point which is more than 30°C higher than that of the ethylene copolymer of said shcath component,
the content of said comonomer is greater than 0.1 mole percent; and
the weight percentage of said heat-bondable fiber in said non-woven fabric is at least 15 weight percent,
characterised in that
the melt index value of said sheath component is 1 to 50 g/10 minutes as measured by the ASTM D-1238(E),
the content of said comonomer is in a range of more than 0.79 mole percent, but no more than 5.0 mole percent, and
the fiber forming polymer consisting of polypropylene, nylon 6, or polyethylene terephthalate.

## Patentansprüche

1. Ein nichtgewebter Stoff aus einer wärmebindbaren Stapelfaser in Form einer zusammengesetzter Faser mit Kern und Hülle, mit
einer Kernkomponente und eine Hüllenkomponente, die den Umfang der Kernkomponente überdeckt,
wobei die Hüllenkomponente aus einem Äthylencopolymer gebildet ist, das aus Äthylen und einem anderen Comonomer besteht, wobei das Comonomer aus mindestens einem der Stoffe besteht, die aus der Klasse ausgewählt sind, die aus einer ungesättigten Carboxylsäure, einem Derivat von dieser ungesättigten Carboxylsäure und aus einem Carboxylsäureanhydrid der ungesättigten Carboxylsäure besteht,
wobei die zusammengesetzte Faser des Typs von Kern und Hülle eine Einzelfaserstärke von weniger als 8 Deniers besitzt,
der nichtgewebte Stoff mit der hitzebindbaren Faser bei einer Temperatur unterhalb des Schmelzpunktes der Kernkomponente wärmebehandelt wird,
die Kernkomponente aus einem faserbildenden Polymer besteht, wobei dieses faserbildende Polymer einen Schmelzpunkt besitzt, der mehr als 30° größer als der des Äthylencopolymers in der Hüllenkomponente ist,
der Anteil des Comonomers größer als 0,1 Moleprozent ist, und
der Gewichtsanteil der wärmebindbaren Faser in dem nichtgewebten Stoff zumindest 15 Gewichtsprozent besitzt,
dadurch gekennzeichnet, daß
der Schmelzindexwert der Hüllenkomponente zwischen 1 und 50 g/10 Minuten gemessen durch ASTM D-1238(E) ist,
der Anteil des Comonomers in dem Bereich von mehr als 0,79 Moleprozent, nicht jedoch mehr als 5,0 Moleprozent liegt, und
das faserbildende Polymer aus Polyäthylen-Terephthalat, Polypropylen oder Nylon 6 besteht.

## Revendications

1. Non-tissé composé de fibres coupées thermo-liables sous la forme de fibres composites du type à âme et gaine comprenant
un composant d'âme et un composant de gaine qui recouvre la périphérie dudit composant d'âme,
ledit composant de gaine étant formé d'un copolymère d'éthylène composé d'éthylène et d'un autre comonomère qui est constitué par au moins un membre choisi dans le groupe consistant en les acides carboxyliques insaturés, les dérivés desdits acides carboxyliques insaturés et les anhydrides desdits acides carboxyliques insaturés,
lesdites fibres composites du type à âme et gaine ayant un degré homogène de finesse de fibres de moins de 8 deniers,
ledit non-tissé contenant lesdites fibres thermo-liables et étant traité thermiquement à une température inférieure au point de fusion du composant d'âme,
ledit composant d'âme consistant en un polymère formant des fibres,
ledit polymère formant des fibres ayant un point de fusion qui est supérieur de plus de 30°C à celui du copolymère d'éthylène dudit composant de gaine,
la teneur en ledit comonomère étant supérieure à 0,1% en moles, et
le pourcentage en poids desdites fibres thermo-liables dans ledit non-tissé étant d'au moins 15% en poids,
caractérisé en ce que
l'indice d'écoulement à l'état fondu dudit composant de gaine a une valeur de 1 à 50 g/10 min, mesuré selon la norme ASTM D-1238(E),
la teneur en ledit comonomère est supérieure à 0,79% en moles, mais ne dépasse pas 5,0% en moles, et
le polymère formant des fibres est constitué par du polypropylène, du nylon-6 ou du polytéréphtalate d'éthylène.
